# EUROPEAN PATENT SPECIFICATION

(11) **EP 2 499 268 B1**
(45) Date of publication and mention of the grant of the patent: **04.01.2017**
(21) Application number: 10782233.0
(22) Date of filing: 15.11.2010
(51) Int. Cl.: C22C 1/05, C22C 29/08

(54) **CEMENTED CARBIDE AND PROCESS FOR PRODUCING THE SAME**
Hartmetall und Verfahren zu seiner Herstellung
CARBURE METALLIQUE ET PROCEDE POUR SA PRODUCTION

(30) Priority: 13.11.2009 GB 0919857
(43) Date of publication of application: 19.09.2012
(73) Proprietor: Element Six GmbH, 36151 Burghaun (DE)
(72) Inventor: KONYASHIN, Igor Yuri, 36151 Burghaun (DE); RIES, Bernd Heinrich, 36151 Burghaun (DE); LACHMANN, Frank Friedrich, 36151 Burghaun (DE)
(74) Representative: Mitchell, Matthew Benedict David
(86) International application number: PCT/EP2010/067463
(87) International publication number: WO 2011/058167

(56) References cited:
- EP-A1- 1 281 670
- EP-A1- 2 011 890
- JP-A- 2005 200 671
- US-A- 3 451 791
- US-A1- 2005 005 732
- KONYASHIN, I. ET AL: "Near - nano WC -Co hardmetals: Will they substitute conventional coarse-grained mining grades?", INTERNATIONAL JOURNAL OF REFRACTORY METALS & HARD MATERIALS , 28(4), 489-497 CODEN: IRMME3; ISSN: 0958-0611, 2010, XP009146295,
- YOURONG LIU ET AL: "Near-nanostructured WC-18 pct Co coatings with low amounts of non-WC carbide phase: Part II. Hardness and resistance to sliding and abrasive wear", METALLURGICAL AND MATERIALS TRANSACTIONS A, SPRINGER-VERLAG, NEW YORK, vol. 33, no. 1, 1 January 2002 (2002-01-01), pages 159-164, XP019693964, ISSN: 1543-1940
- ZHAO ET AL: "Effects of scale combination and contact condition of raw powders on SPS sintered near-nanocrystalline WC-Co alloy", MATERIALS SCIENCE AND ENGINEERING A: STRUCTURAL MATERIALS:PROPERTIES, MICROSTRUCTURE & PROCESSING, LAUSANNE, CH, vol. 473, no. 1-2, 2 January 2008 (2008-01-02), pages 323-329, XP022406205, ISSN: 0921-5093, DOI: DOI:10.1016/J.MSEA.2007.04.094

## Description

### Field

This invention relates to cemented carbide comprising tungsten carbide (WC) grains with mean grain size of below 0.3 micron and to methods of making such cemented carbide.

### Background

There is a general trend in the cemented carbide industry to produce WC-Co materials with WC mean grain size as low as possible, in particular having a grain size in the region of nanomaterials (grain size smaller than 0.1 micron or 100 nm). WC-Co hardmetals with a WC mean grain size of nearly 0.2 micron, produced from WC powders with a mean grain size of below 0.3 micron are designated as "near-nano cemented carbides" or "near-nano hardmetals" (see for example M.Brieseck, I.Hünsche et al. "Optimised sintering and grain-growth inhibition of ultrafine and near-nano hardmetals". Proc. Int. Conf. PM2009, Copenhagen, EPMA). The near-nano cemented carbides are found to possess an improved combination of hardness and fracture toughness compared to conventional ultra-fine grained hardmetals with mean grain size of 0.3 to 0.8 µm.

EP1413637 discloses cemented carbide with improved toughness for oil and gas applications. The cemented carbide contains 8 wt.% to 12 wt.% Co+Ni, 1 wt.% to 2 wt.% Cr and 0.1 wt.% to 0.3 wt.% Mo, the rest being WC. All the WC grains are smaller than 1 micron and the magnetic Co content is between 80% and 90% of the chemically determined Co. The mean grain size of WC powder is nearly 0.8 micron. EP1413637 does not, however, provide information on the composition of near-nano cemented carbides.

EP1043412 discloses a method for making submicron cemented carbide with increased toughness. The WC grains of the WC powder according to EP1043412 are coated with Cr and Co prior to mixing. The WC grains have an average grain size in the range of 0.2 micron to 1.0 micron, preferably 0.6 micron to 0.9 micron. EP1043412 provides no information with respect to the fabrication of near-nano cemented carbides.

JP2005200671 describes a cemented carbide alloy having a d10, d50 and d90 particle diameter of 0.15 micron or less, 0.35 micron or less and 0.6 micron or less, respectively measured from the particle size distribution.

Konyashin et. al., "Near-nano WC-Co hardmetals: Will they substitute conventional coarse-grained mining grades", International Journal of Refractory Metals & Hard Materials, 28(4) 489-497 describes a cemented carbide.

There are three major problems with respect to the production of near-nano cemented carbide from nano or near-nano WC powders. The first problem is related to the very intensive WC grain growth which occurs during the liquid-phase sintering of WC-Co when nano or near-nano powders are used. The WC grain growth can be suppressed by use of grain growth inhibitors, mainly chromium and vanadium carbides, however, only at the expense of cemented carbide fracture toughness.

The second problem is related to the very high activity of WC-Co green articles pressed from powder mixtures comprising nano or near-nano WC powders with respect to deviations of carbon content in the gas atmospheres during sintering. If the carbon potential in the sintering furnace is slightly above a certain level, free carbon forms in the microstructure of near-nano cemented carbides. If the carbon potential in the sintering furnace is slightly below a certain level, the decarburisation of near-nano cemented carbide can easily occur, leading to the formation of eta-phases (Co3W3C or Co6W6C) in the microstructure of near-nano cemented carbides.

The third problem is related to the necessity for fine regulation of the carbon content in powder WC-Co mixtures obtained from nano or near-nano powders. In the conventional practice of carbide fabrication, the carbon content is varied by addition of either W metal or carbon black. However, in the case of near-nano cemented carbide even insignificant additions of W metal or carbon black are found to lead in defects of the microstructure, such as fields enriched with Co (Co lakes) and/or abnormally large WC grains. Moreover, when taking into account that the powder WC-Co mixtures containing near-nano WC are heavily oxidised, the mixtures have to be annealed in a reducing gas atmosphere.

When taking into account the above-mentioned problems, there is a need for new compositions of near-nano cemented carbide having further enhanced carbon content indicated by the cemented carbide magnetic saturation. Also, a new method of regulation of carbon content in green parts of near-nano cemented carbides is needed.

There is a need to provide near-nano cemented carbide with an improved combination of hardness, fracture toughness and wear-resistance.

### Summary

According to a first aspect there is provided a process for production of cemented carbide comprising WC grains, 3 wt.% to 20 wt.% binder selected from Co or Co and Ni and grain growth inhibitors wherein the WC mean grain size lies in the range of 180 nm and 230 nm, at least 10±2 % WC grains are finer than 50 nm and 7±2% WC grains have a size from 50 to 100 nm, the process including the following stages:
- milling WC powder with specific surface area (BET) of 3.0 m²/g or higher with binder and grain-growth inhibitors;
- pressing green parts;
- pre-sintering the green parts in H2 at 400°C to 900°C (degrees Centigrade) for 5 min. to 30 min;
- sintering in vacuum at temperatures of 1340°C to 1410°C for 3 min to 20 min; and
- HIP-sintering in Ar at pressures of 40 to 100 bar at temperatures of 1340°C to 1410°C for 1 to 20 min.
It has surprisingly been found that the carbon content in the green articles of the near-nano cemented carbides with the composition and WC grain sizes mentioned above according to the first aspect of the present invention can be precisely regulated by pre-sintering in pure hydrogen at temperatures of 400°C to 900°C and finally sintered in vacuum and Ar under pressure.

As an option, the binder includes tungsten dissolved therein and the concentration of tungsten dissolved in the binder lies in the range of 14 wt.% to 25 wt.%, which is indicated by the magnetic moment/unit wt. of the cemented carbide according to the equations: ${σ}_{cc} = {σ}_{B} B / 100$ ${σ}_{B} = {σ}_{Co} - 0.275 {M}_{w} ,$ where σ_{cc} is the magnetic moment of the cemented carbide in units of micro-Tesla times cubic metre per kilogram, σ_{Co} is the magnetic moment of pure cobalt in units of micro-Tesla times cubic metre per kilogram, B is the binder fraction in the cemented carbide in wt.%, σ_{B} is the magnetic moment of the binder in units of micro-Tesla times cubic metre per kilogram and M_{w} is the concentration of tungsten dissolved in the binder in wt.%.

As an option, the concentration of tungsten dissolved in the binder lies in the range of 16 wt.% to 25 wt.%.

As a further option, the concentration of tungsten dissolved in the binder lies in the range of 18 wt.% to 25 wt.%.

The grain growth inhibitor content with respect to the binder optionally comprises 3 wt.% to 11 wt.% Cr and 1 wt.% to 4 wt.% V.

As a further option, the grain growth inhibitor content with respect to the binder content comprises 3 wt.% toll wt.% Cr; 1 wt.% to 4 wt.% V; 0.1 wt.% to 8 wt.% Zr; 0.1 wt.% to 5 wt.% Ta and/or 0.1 wt.% to 10.0 wt.% Mo.

As an option, the coercive field strength of the cemented carbide lies in the range of 32 kA/m to 72 kA/m (kilo Amperes per metre).

The toughness-hardness coefficient obtained by multiplication of indentation fracture toughness in MPa.m^{½} and Vickers hardness in GPa is optionally above 180. As a further option, the toughness-hardness coefficient obtained by multiplication of indentation fracture toughness in MPa.m^{½} and Vickers hardness in GPa is optionally above 200.

The cemented carbide optionally exhibits wear measured according to the ASTM B611 test in cm³/rev. of below 0.12Y 10⁻⁵ where Y is the binder fraction, in wt.%.

The cemented carbide optionally comprises neither free carbon nor eta-phases.

The grain growth inhibitors are optionally present in the form of solid solution in the binder.

The grain growth inhibitors are optionally present in form of carbides.

Such near-nano cemented carbides have an exceptionally high combination of hardness, fracture toughness and wear-resistance.

### Drawing captions

Embodiments will be described by way of non-limiting examples, and with reference to the accompanying drawings in which:
FIG 1A shows an FE-SEM image of the microstructure of the near-nano cemented carbide according Example 1, FIG 1B shows the corresponding FE-SEM image after computer image processing, and FIG 1C shows corresponding light-microscopy image.
FIG 2A shows a graph of the wear of the near-nano (NN) cemented carbide according to Example 1 in comparison with those of conventional ultra-fine (UF) cemented carbides (WC mean grain size of nearly 0.8 µm) with 10 and 7 % Co. FIG 2B shows a graph of the corresponding fracture toughness.
FIG 3 shows the microstructure of the near-nano cemented carbide according Example 2 (light-microscopy).
FIG 4A shows a graph of the wear of the near-nano (NN) cemented carbide according to Example 2 in comparison with those of conventional ultra-fine (UF) cemented carbide (WC mean grain size of nearly 0.8 µm) with 5 % Co. FIG 4B shows a graph of the corresponding fracture toughness.

### Detailed Description

Measurements of magnetic properties are widely used in the cemented carbide industry. Both coercive force and magnetic moment are measured for these purposes. The coercive force indicates the thickness of Co interlayers among WC grains and consequently WC mean grain size. The amount of tungsten dissolved in the Co-based binder can be assessed by measurement of magnetic moment or magnetic saturation of cemented carbides because the saturation value of Co decreases linearly with the addition of tungsten in solution (see B. Roebuck & E. Almond., Int. Mater Rev., 33(1988)90-110). It is well known that the concentration of tungsten dissolved in the binder increases when decreasing the total carbon content, so that the magnetic moment shows indirectly the total carbon content in cemented carbides. The equation indicating the dependence of magnetic moment of cemented carbide on the concentration of tungsten dissolved in the binder is the following (see. B. Roebuck. Int. J, Refractory Met. Hard Mater., 14(1996)419-424): σB = σCo-0.275 Mw, where σCo is the magnetic moment of pure cobalt in units of micro-Tesla times cubic metre per kilogram, σB is the magnetic moment of the binder in units of micro-Tesla times cubic metre per kilogram and Mw is the concentration of tungsten dissolved in the binder in wt.%.

It is well known that in WC-Co cemented carbides not containing η-phase (Co3W3C or Co6W6C) when the total carbon content decreases the concentration of tungsten dissolved in the binder strongly increases, which is indicated by decreasing the magnetic moment. In such cemented carbides the WC grains in the microstructure become significantly finer compared to cemented carbides with medium or high total carbon content and consequently with lower concentrations of tungsten dissolved in the binder. In other words, high concentrations of tungsten dissolved in the binder act as "a grain growth inhibitor" suppressing the process of re-crystallisation of fine grain WC fraction and growth of large WC single-crystals (see I.Konyashin, et al. Int. J. Refractory Met. Hard Mater., 27(2009)234-243). The major advantage of employing high concentrations of tungsten dissolved in the binder as "a grain growth inhibitor" compared to conventional grain growth inhibitors (Cr, V, etc.) is that the fracture toughness of extremely fine-grained with high concentrations of tungsten dissolved in the binder does not decrease or decreases to a lesser extent compared to cemented carbides with medium or low concentration of tungsten dissolved in the binder, but containing a large amount of the conventional grain growth inhibitors. This is related to the fact that the conventional grain growth inhibitors segregate at WC-Co interfaces leading to their "weakening" and a decreased fracture toughness (see e.g. S. Lay et al Int. J. Refractory Met. Hard Mater., 20(2002)61-69), whereas in the cemented carbides with high concentration of tungsten dissolved in the binder the WC-Co interfaces remain unchanged (see I.Konyashin et al. Int. J. Refractory Met. Hard Mater., 28(2010)228-237). Therefore, it is possible to achieve higher combinations of hardness and fracture toughness of near-nano cemented carbides by using high concentrations of tungsten dissolved in the binder. The use of high concentration of tungsten dissolved in the binder can be combined with the employment of a certain type and amount of conventional grain growth inhibitors.

It has surprisingly been found that when the concentration of tungsten dissolved in the binder varies from 14 wt.% to 25 wt.%, preferably 16 wt.% to 25 wt.%, most preferably 18 wt.% to 25 wt.% the hardness of near-nano cemented carbides can be increased without loosing their fracture toughness. In other words, the near-nano cemented carbides with a certain combinations of microstructure characteristics and with high concentrations of tungsten dissolved in the binder possess an unexpectedly high combination of hardness and fracture toughness as well as very high wear-resistance. The concentration of tungsten dissolved in the binder should be on the one hand as high as possible, but on the other hand be limited by the fact that, at a certain concentration of tungsten dissolved in the binder, eta-phases (Co3W3C and Co6W6C) form in the microstructure. The formation of eta-phases is very undesirable, as it leads to a dramatic decrease of the cemented carbide transverse rupture strength.

### Examples

Embodiments of the invention are described in more detail with reference to the examples below, which are not intended to limit the invention.

### Example 1

Tungsten carbide powder (4NP0 from H.C.Starck™, Germany) with the specific surface (BET) of 4.0 m²/g measured according to the ASTM 3663 standard and carbon content of 6.14 wt.%, was blended with about 10 wt.% cobalt powder, wherein the Co grains had an average grain size of about 1 micron, 0.8 wt.% Cr3C2, 0.3 wt.% VC, 0.5 wt.% Mo2C, 0.1 wt.% TaC and 0.1 wt.% ZrC. The blend was produced by milling the powders together for 24 hrs by means of a ball mill in a milling medium consisting of hexane with 2 wt.% paraffin wax, and using a powder-to-ball ratio of 1:6. After drying the blend, samples of various sizes including those for examining transverse rupture strength (TRS) according to the ISO 3327-1982 standard and wear-resistance according to the ASTM B611-85 standard were pressed and heat-treated in hydrogen at 700°C centigrade for 20 min. The green bodies were then sintered at 1370°C for 20 min, including a 10 minute vacuum sintering stage and a 10 minute high isostatic pressure (HIP) sintering stage carried out in an argon atmosphere at a pressure of 50 bar.

Metallurgical cross-sections were made and examined by use of a light microscope and a FE-SEM. FIG 1A, FIG 1B and FIG 1C show the microstructure of the cemented carbide. It clearly seen that there is neither free-carbon nor η-phase in the microstructure and it is fine and uniform. The microstructure obtained on the FE-SEM was analysed using the AnalySIS™ software from the company "Soft Imaging System™" (SIS). The WC mean grain size was found to be equal to 0.20 micron, the percentage of grains finer than 50 nm was found to be 9.6% and that of grains of 50 to 100 nm was found to be 7.0%. The properties of the cemented carbide were as follows: density - 14.24 g/cm³, TRS - 3300 MPa, HV20 - 20.5 GPa, coersivity - 40.6 kA/m, magnetic moment - 1,1 µT m³/kg, fracture toughness - 9.9 MPa.m^{½}, wear - 1.0 10⁻⁵ cm³/rev. Thus, the toughness-hardness coefficient obtained by multiplication of fracture toughness in MPa.m^{½} and Vickers hardness in GPa is equal to roughly 203. The concentration of tungsten dissolved in the binder calculated on the basis of the magnetic moment value is equal to 18.5 wt.%. FIG 2A and FIG 2B show the wear-resistance and fracture toughness of the near-nano cemented carbide in comparison with conventional ultra-fine grades with WC mean grain size of 0.8 micron with 10% Co and 7% Co. The microstructure of the conventional grades does comprise grains finer than 100 nm, they contain 0.3 wt.% VC and 0.2 wt.% Cr3C2 and the concentration of tungsten dissolved in the binder of these grades was below 10 wt%. It is clearly seen that the wear-resistance of the near-nano cemented carbide is significantly higher than that of the conventional grades, which is achieved by only an insignificant decrease in fracture toughness compared to the conventional grade with 10%Co, and higher fracture toughness compared to the conventional grade with 7% Co. The hardness of the ultra-fine grade with 7% Co is 17.0 GPa and its fracture toughness is 9.2 MPa.m^{1/2}, so that the toughness-hardness coefficient of this grade is equal to 156, which is significantly lower than that of the new near-nano cemented carbide. The hardness of the ultra-fine grade with 10% Co is 15.0 GPa and its fracture toughness is 10.7 MPa.m^{1/2}, so that the toughness-hardness coefficient of this grade is equal to 160, which is significantly lower than that of the new near-nano cemented carbide.

### Example 2

Tungsten carbide powder (4NP0 from H.C.Starck™, Germany) with the specific surface (BET) of 4.0 m²/g measured according to the ASTM 3663 standard and carbon content of 6.14 wt.%, was blended with about 5 wt.% cobalt powder, wherein the Co grains had an average grain size of about 1 micron, 0.4 wt.% Cr3C2, 0.15 wt.% VC, 0.25 wt.% Mo2C, 0.05 wt.% TaC and 0.05 wt.% ZrC. The blend was produced by milling the powders together for 24 hours by means of a ball mill in a milling medium consisting of hexane with 2 wt.% paraffin wax, and using a powder-to-ball ratio of 1:6. After drying the blend, samples of various sizes including those for examining transverse rupture strength (TRS) according to the ISO 3327-1982 standard and wear-resistance according to the ASTM B611-85 standard were pressed and heat-treated in hydrogen at 700°C centigrade for 20 min. The green bodies were then sintered at 1390°C for 20 min, including a 10 minute vacuum sintering stage and a 10 minute high isostatic pressure (HIP) sintering stage carried out in an argon atmosphere at a pressure of 50 bar.

Metallurgical cross-sections were made and examined by use of a light microscope. FIG 3 shows the microstructure of the cemented carbide. It can clearly be seen that there is neither free-carbon nor eta-phase in the microstructure and it is fine and uniform; the cross-sections were also examined on the FE-SEM. The microstructure obtained on the FE-SEM was analysed using the AnalySIS™ software from the company "Soft Imaging System^{™}" (SIS). The WC mean grain size was found to be equal to 0.19 micron, the percentage of grains finer than 50 nm was found to be 9.0% and that of grains of 50 to 100 nm was found to be 6.4%.

The properties of the cemented carbide are the following: density - 14.98 g/cm³, TRS - 2500 MPa, HV20 - 22.5 GPa, coersivity - 43.0 kA/m, magnetic moment - 0,5 µT m³/kg, fracture toughness - 9.2 MPa m^{½}, wear - 1.9 10⁻⁶ cm³/rev. Thus, the toughness-hardness coefficient obtained by multiplication of fracture toughness in MPa.m^{½} and Vickers hardness in GPa is equal to roughly 207. The concentration of tungsten dissolved in the binder calculated on the basis of the magnetic moment value is equal to 22.2 wt.%. FIG 4A and FIG 4B show the wear and fracture toughness of the near-nano cemented carbide in comparison with a conventional ultra-fine grade with WC mean grain size of 0.8 µm with 5% Co. The microstructure of the conventional grade does comprise grains finer than 100 nm, it contains 0.2 wt.% VC and 0.1 wt.% Cr3C2 and the concentration of tungsten dissolved in the binder of the grade was below 9 wt%. It is clearly seen that the wear-resistance of the new near-nano cemented carbide is significantly higher than that of the conventional grade, which is achieved without losing fracture toughness. The hardness of the conventional ultra-fine grade with 5% Co is 17.8 GPa and its fracture toughness is 9.0 MPa.m^{1/2}, so that the toughness-hardness coefficient of this grade is equal to 160, which is significantly lower than that of the near-nano cemented carbide.

## Claims

1. A process for production of cemented carbide comprising WC grains, 3 wt.% to 20 wt.% binder selected from Co or Co and Ni and grain growth inhibitors wherein the WC mean grain size lies in the range of 180 nm and 230 nm, at least 10±2 % of the WC grains are finer than 50 nm and 7±2% WC grains have a size from 50 to 100 nm, the process including the following stages:
• milling WC powder with specific surface area (BET) of 3.0 m²/g or higher with binder and grain-growth inhibitors;
• pressing green parts;
• pre-sintering the green parts in H2 at 400°C to 900°C for 5 to 30 min;
• sintering in vacuum at temperatures of 1340°C to 1410°C for 3 min to 20 min; and
• HIP-sintering in Ar at pressures of 40 to 100 bar at temperatures of 1340°C to 1410°C for 1 to 20 min.

2. A process according to claim 1 wherein the concentration of tungsten dissolved in the binder lies in the range of 14 wt.% to 25 wt.%, which is indicated by the magnetic moment/unit wt. of the cemented carbide according to the equations: ${σ}_{cc} = {σ}_{B} B / 100$ ${σ}_{B} = {σ}_{Co} - 0.275 {M}_{w} ,$ where σ_{cc} is the magnetic moment of the cemented carbide in units of micro-Tesla times cubic metre per kilogram, σ_{Co} is the magnetic moment of pure cobalt in units of micro-Tesla times cubic metre per kilogram, B is the binder fraction in the cemented carbide in wt.%, σ_{B} is the magnetic moment of the binder in units of micro-Tesla times cubic metre per kilogram and M_{w} is the concentration of tungsten dissolved in the binder in wt.%.

3. A process according to any preceding claim wherein the concentration of tungsten dissolved in the binder lies in the range of 16 wt.% to 25 wt.%.

4. A process according to any preceding claim wherein the concentration of tungsten dissolved in the binder lies in the range of 18 wt.% to 25 wt.%

5. A process according to any preceding claim wherein the grain growth inhibitor content with respect to the binder comprises 3 wt.% to 11 wt.% Cr and 1 wt.% to 4 wt.% V.

6. A process according any preceding claim wherein the grain growth inhibitor content with respect to the binder content comprises 3 wt.% to 11 wt.% Cr; 1 wt.% to 4 wt.% V; 0.1 wt.% to 8 wt.% Zr; 0.1 wt.% to 5 wt.% Ta and/or 0.1 wt.% to 10.0 wt.% Mo.

7. A process according to any preceding claim wherein the coercive field strength of the cemented carbide lies in the range of 32 kA/m to 72 kA/m.

8. A process according to any preceding claim wherein the toughness-hardness coefficient obtained by multiplication of indentation fracture toughness in MPa.m^{½} and Vickers hardness in GPa lies above 180.

9. A process according to any preceding claim wherein the toughness-hardness coefficient obtained by multiplication of indentation fracture toughness in MPa.m^{½} and Vickers hardness in GPa lies above 200.

10. A process according to any preceding claim wherein the cemented carbide exhibits wear measured according to the ASTM B611 test in cm³/rev. of below 0.12Y 10⁻⁵, where Y is the binder fraction, in wt.%.

11. A process according to any preceding claim wherein the cemented carbide comprises neither free carbon nor eta-phases.

12. A process according to any preceding claim wherein the grain growth inhibitors are present in form of solid solution in the binder.

13. A process according to any one of claims 1 to 11, wherein the grain growth inhibitors are present in form of carbides.

## Patentansprüche

1. Ein Verfahren zur Herstellung von Hartmetall, umfassend WC-Körner, 3 Gew.-% bis 20 Gew.-% Bindemittel, ausgewählt aus Co oder Co und Ni, und Kornwachstumsinhibitoren, wobei die durchschnittliche Korngröße des WC im Bereich von 180 nm und 230 nm liegt, mindestens 10 ± 2% der WC-Körner feiner sind als 50 nm und 7 ± 2% der WC-Körner eine Größe von 50 bis 100 nm aufweisen, wobei das Verfahren die folgenden Schritte beinhaltet:
• Mahlen von WC-Pulver mit spezifischer Oberfläche (BET) von 3,0 m²/g oder höher mit Bindemittel und Kornwachstumsinhibitoren;
• Pressen von Grünkörpern;
• Vorsintern der Grünkörper in H2 bei 400°C bis 900°C für 5 bis 30 Min.;
• Sintern im Vakuum bei Temperaturen von 1340°C bis 1410°C für 3 Min. bis 20 Min.; und
• HIP-Sintern in Ar bei Drücken von 40 bis 100 bar bei Temperaturen von 1340°C bis 1410°C für 1 bis 20 Min.

2. Ein Verfahren gemäß Anspruch 1, wobei die Konzentration von Wolfram, das in dem Bindemittel gelöst ist, im Bereich von 14 Gew.-% bis 25 Gew.-% liegt, die durch das magnetische Moment/Einheitsgewicht des Hartmetalls gemäß den Gleichungen angegeben ist: ${σ}_{cc} = {σ}_{B} B / 100$ ${σ}_{B} = {σ}_{Co} - 0 , 275 {M}_{w} ,$ wobei σ_{cc} das magnetische Moment des Hartmetalls in Einheiten von Mikrotesla mal Kubikmeter pro Kilogramm ist, σ_{Co} das magnetische Moment von reinem Kobalt in Einheiten von Mikrotesla mal Kubikmeter pro Kilogramm ist, B der Bindemittelanteil im Hartmetall in Gew.-% ist, σ_{B} das magnetische Moment des Bindemittels in Einheiten von Mikrotesla mal Kubikmeter pro Kilogramm ist und M_{W} die Konzentration von Wolfram, das im Bindemittel gelöst ist, in Gew.-% ist.

3. Ein Verfahren gemäß einem der vorangehenden Ansprüche, wobei die Konzentration von Wolfram, das in dem Bindemittel gelöst ist, im Bereich von 16 Gew.-% bis 25 Gew.-% liegt.

4. Ein Verfahren gemäß einem der vorangehenden Ansprüche, wobei die Konzentration von Wolfram, das im Bindemittel gelöst ist, im Bereich von 18 Gew.-% bis 25 Gew.-% liegt.

5. Ein Verfahren gemäß einem der vorangehenden Ansprüche, wobei der Kornwachstumsinhibitor-Gehalt, bezogen auf das Bindemittel, 3 Gew.-% bis 11 Gew.-% Cr und 1 Gew.-% bis 4 Gew.-% V umfasst.

6. Ein Verfahren gemäß einem der vorangehenden Ansprüche, wobei der Kornwachstumsinhibitor-Gehalt, bezogen auf den Bindemittelgehalt, 3 Gew.-% bis 11 Gew.-% Cr; 1 Gew.-% bis 4 Gew.-% V; 0,1 Gew.-% bis 8 Gew.-% Zr; 0,1 Gew.-% bis 5 Gew.-% Ta und/oder 0,1 Gew.-% bis 10,0 Gew.-% Mo umfasst.

7. Ein Verfahren gemäß einem der vorangehenden Ansprüche, wobei die Koerzitivfeldstärke des Hartmetalls im Bereich von 32 kA/m bis 72 kA/m liegt.

8. Ein Verfahren gemäß einem der vorangehenden Ansprüche, wobei der Zähigkeits-Härte-Koeffizient, erhalten durch Multiplikation der Eindruck-Bruchzähigkeit in MPa•m^{½} und Vickershärte in GPa, über 180 liegt.

9. Ein Verfahren gemäß einem der vorangehenden Ansprüche, wobei der Zähigkeits-Härte-Koeffizient, erhalten durch Multiplikation der Eindruck-Bruchzähigkeit in MPa•m^{½} und Vickershärte in GPa, über 200 liegt.

10. Ein Verfahren gemäß einem der vorangehenden Ansprüche, wobei das Hartmetall Verschleiß, gemessen gemäß dem ASTM B611 Test in cm³/rev., von unter 0,12Y 10⁻⁵ aufweist, wobei Y der Bindemittelanteil in Gew.-% ist.

11. Ein Verfahren gemäß einem der vorangehenden Ansprüche, wobei das Hartmetall weder freien Kohlenstoff noch eta-Phasen umfasst.

12. Ein Verfahren gemäß einem der vorangehenden Ansprüche, wobei die Kornwachstumsinhibitoren in Form einer festen Lösung im Bindemittel vorliegen.

13. Ein Verfahren gemäß einem der Ansprüche 1 bis 11, wobei die Kornwachstumsinhibitoren in Form von Carbiden vorliegen.

## Revendications

1. Procédé de production de carbure cémenté comprenant des grains de WC, 3% en poids à 20% en poids d'un liant choisi parmi le Co ou le Co et le Ni et des inhibiteurs de croissance de grain où la taille moyenne de grain de WC se trouve dans la plage allant de 180 nm à 230 nm, au moins 10 ± 2% des grains de WC sont plus fins que 50 nm et 7 ± 2% de grains de WC ont une taille allant de 50 à 100 nm, le procédé comportant les étapes suivantes qui consistent :
• à broyer la poudre de WC ayant une surface spécifique (BET) de 3,0 m²/g ou plus avec un liant et des inhibiteurs de croissance de grain ;
• à presser des parties vertes ;
• à pré-fritter les parties vertes dans le H2 à une température comprise entre 400°C et 900°C pendant 5 à 30 min ;
• à effectuer un frittage sous vide à des températures comprises entre 1340°C et 1410°C pendant 3 min à 20 min ; et
• à effectuer un frittage HIP dans l'Ar à des pressions allant de 40 à 100 bar à des températures comprises entre 1340°C et 1410°C pendant 1 à 20 min.

2. Procédé selon la revendication 1, dans lequel la concentration de tungstène dissous dans le liant se trouve dans la plage allant de 14% en poids à 25% en poids, qui est indiquée par le moment magnétique/le poids unitaire du carbure cémenté selon les équations : ${σ}_{cc} = {σ}_{B} B / 100$ ${σ}_{B} = {σ}_{Co} - 0 , 275 {M}_{w} ,$ où σ_{cc} est le moment magnétique du carbure cémenté en unités de micro-Tesla fois mètre cube par kilogramme, σ_{Co} est le moment magnétique de cobalt pur en unités de micro-Tesla fois mètre cube par kilogramme, B est la fraction de liant dans le carbure cémenté en % en poids, σ_{B} est le moment magnétique du liant en unités de micro-Tesla fois mètre cube par kilogramme et M_{w} est la concentration de tungstène dissous dans le liant en % en poids.

3. Procédé selon l'une des revendications précédentes, dans lequel la concentration de tungstène dissous dans le liant se trouve dans la plage allant de 16% en poids à 25% en poids.

4. Procédé selon l'une des revendications précédentes, dans lequel la concentration de tungstène dissous dans le liant se trouve dans la plage allant de 18% en poids à 25% en poids.

5. Procédé selon l'une des revendications précédentes, dans lequel la teneur en inhibiteur de croissance de grain par rapport au liant comprend 3% en poids à 11% en poids de Cr et 1% en poids à 4% en poids de V.

6. Procédé selon l'une des revendications précédentes, dans lequel la teneur en inhibiteur de croissance de grain par rapport à la teneur en liant comprend 3% en poids à 11% en poids de Cr ; 1% en poids à 4% en poids de V ; 0,1% en poids à 8% en poids de Zr ; 0,1% en poids à 5% en poids de Ta et/ou 0,1% en poids à 10,0% en poids de Mo.

7. Procédé selon l'une des revendications précédentes, dans lequel le champ coercitif du carbure cémenté se trouve dans la plage allant de 32 kA/m à 72 kA/m.

8. Procédé selon l'une des revendications précédentes, dans lequel le coefficient de ténacité-dureté obtenu par multiplication de la ténacité à la rupture par indentation en MPa.m^{1/2} et de la dureté Vickers en GPa se trouve au-dessus de 180.

9. Procédé selon l'une des revendications précédentes, dans lequel le coefficient de ténacité-dureté obtenu par multiplication de la ténacité à la rupture par indentation en MPa.m^{1/2} et de la dureté Vickers en GPa se trouve au-dessus de 200.

10. Procédé selon l'une des revendications précédentes, dans lequel le carbure cémenté présente une usure mesurée selon le test ASTM B611 en cm³/rev inférieure à 0,12Y 10⁻⁵, où Y est la fraction de liant, en % en poids.

11. Procédé selon l'une des revendications précédentes, dans lequel le carbure cémenté ne comprend ni du carbone libre ni des phases eta.

12. Procédé selon l'une des revendications précédentes, dans lequel les inhibiteurs de croissance de grain sont présents sous forme d'une solution solide dans le liant.

13. Procédé selon l'une quelconque des revendications 1 à 11, dans lequel les inhibiteurs de croissance de grain sont présents sous forme de carbures.
